



US005379004A

**United States Patent** [19]

Marusawa et al.

[11] **Patent Number:** 5,379,004[45] **Date of Patent:** Jan. 3, 1995[54] **HIGH FREQUENCY-USE  
NON-RECIPROCAL CIRCUIT ELEMENT**

[75] Inventors: Hiroshi Marusawa; Takashi Kawanami; Takehiro Kounoike; Kunisaburo Tomono, all of Nagaokakyō, Japan

[73] Assignee: Murata Manufacturing Co., Ltd., Kyoto, Japan

[21] Appl. No.: 101,895

[22] Filed: Aug. 2, 1993

[30] **Foreign Application Priority Data**

Aug. 5, 1992 [JP] Japan ..... 4-208963

[51] Int. Cl.<sup>6</sup> ..... H01P 1/387[52] U.S. Cl. ..... 333/1.1; 333/24.1;  
156/89; 264/61

[58] Field of Search ..... 333/1.1, 24.1, 24.2

[56] **References Cited****U.S. PATENT DOCUMENTS**

5,068,629 11/1991 Nishikawa et al. ..... 333/1.1

**FOREIGN PATENT DOCUMENTS**0381412 1/1990 European Pat. Off. ....  
2266412 10/1993 United Kingdom .**OTHER PUBLICATIONS**

JP 03044011 A. Abstract only.

JP 02060109 A, Abstract only.

Great Britain Search Report dated Nov. 8, 1993.

*Primary Examiner*—Paul Gensler*Attorney, Agent, or Firm*—Ostrolenk, Faber, Gerb & Soffen[57] **ABSTRACT**

A high-frequency-use non-reciprocal circuit element comprises a high-frequency-use magnetic layer and a plurality of center electrodes arranged therein to intersect with each other while being electrically insulated from each other. The plurality of center electrodes are advantageously embedded in the high-frequency-use magnetic layer or layers to be integrated with the same.

**20 Claims, 7 Drawing Sheets**

Fig. 1



Fig. 2



Fig. 3



Fig. 4



Fig. 5



Fig. 6



Fig. 7



Fig. 8



Fig. 9



Fig. 10



Fig. 11



Fig. 12



Fig. 13 PRIOR ART



## HIGH FREQUENCY-USE NON-RECIPROCAL CIRCUIT ELEMENT

### BACKGROUND OF THE INVENTION

#### 1. Field of the Invention

The present invention relates to a non-reciprocal circuit element which is used in a microwave band, and more particularly, it relates to a structure of a high frequency-use non-reciprocal circuit element which is usable in a circulator, an isolator or the like, for example.

#### 2. Description of the Background Art

In recent years, a high-frequency device is increasingly miniaturized and generalized in a mobile communication system or the like. Thus, it is strongly required to reduce the size and cost of a non-reciprocal circuit element employed therein.

Such a non-reciprocal circuit element includes the so-called lumped parameter non-reciprocal circuit element having a plurality of center electrodes which are arranged to intersect with each other in an electrically insulated state, and high frequency-use magnetic bodies which are arranged on upper and lower sides of the plurality of center electrodes are arranged so that dc magnetic fields are applied to the plurality of center electrodes by permanent magnets, for example. Examples of such an element are a lumped parameter type circulator, an isolator and the like.

An exemplary method of manufacturing the aforementioned high frequency-use non-reciprocal circuit element is now described with reference to FIG. 13. A center electrode 32a is arranged on a discoidal high frequency-use magnetic body 31a. The center electrode 32a radially extends through the center of an upper surface of the high frequency-use magnetic body 31a to reach a side surface of the high frequency-use magnetic body 31a. Then, an insulating film 32a of an insulating material is arranged on the center electrode 32a, and another center electrode 32b is arranged thereon to intersect with the center electrode 32a. An insulating film 32b, a center electrode 32c and an insulating film 33c are successively arranged on the center electrode 32b, and a high frequency-use magnetic body 31b is finally placed on and fixed to such a structural body. Thereafter permanent magnets are arranged on upper and lower sides of the thus-obtained structure, to apply dc magnetic fields to the structural body which is held between the high frequency-use magnetic bodies 31a and 31b.

In order to manufacture such a conventional high frequency-use non-reciprocal circuit element, the center electrodes 32a to 32c are manually arranged alternately with the insulating films 33a to 33c, as described above with reference to FIG. 13. However, it is extremely difficult to manually assemble the center electrodes 32a to 32c, which are reduced to about several millimeters in length with miniaturization of the high frequency-use non-reciprocal circuit element. In a miniature high frequency-use non-reciprocal circuit element, therefore, imperfect assembling such as relative misregistration of the center electrodes 32a to 32c is so frequently caused that it is difficult to obtain a highly reliable high frequency-use non-reciprocal circuit element.

Further, the manufacturing cost for such a conventional circuit element is increased due to frequent imperfect assembling caused by manual assembling.

While the high frequency-use non-reciprocal circuit element requires a relatively large number of components as hereinabove described, it is difficult to reduce the cost therefor due to restriction in cost reduction for the respective components.

### SUMMARY OF THE INVENTION

An object of the present invention is to provide a high frequency-use non-reciprocal circuit element, which can be reduced in size and cost with a structure being improvable in reliability.

According to a broad aspect of the present invention, provided is a high frequency-use non-reciprocal circuit element comprising a high frequency-use magnetic body and a plurality of center electrodes which are included inside the high frequency-use magnetic body and arranged to intersect with each other while in a state being electrically insulated from each other.

Throughout the specification, the term "high frequency-use magnetic body" indicates a magnetic body which is suitable for forming the aforementioned non-reciprocal circuit element in a microwave band. This high frequency-use magnetic body is not restricted to a magnetic body which is obtained by stacking a plurality of magnetic green sheet layers and firing the thus-obtained laminate as described later with reference to embodiments of the present invention, but also includes a magnetic body which is formed by adhering a plurality of previously fired magnetic plates with each other with an adhesive or the like. In any case, the feature of the present invention resides in that the plurality of center electrodes are included within such a high frequency-use magnetic body to make an integrated structure therewith.

The manufacturing method according to the present invention is adapted to prepare a laminate of high frequency-use magnetic layers and a plurality of center electrodes which are alternately stacked so that the center electrodes intersect with each other while in a state being electrically insulated from each other, and to fire the laminate, thereby obtaining a high frequency-use non-reciprocal circuit element. In this case, the unfired high frequency-use magnetic layers which are stacked alternately with the center electrodes can be prepared from previously shaped unfired magnetic green sheets or unfired magnetic layers formed by applying and hardening magnetic paste.

According to another aspect of the present invention, the aforementioned high frequency-use non-reciprocal circuit element is obtained by preparing high frequency-use magnetic plates which are provided with first center electrodes on at least one single major surfaces thereof and bonding such high frequency-use magnetic plates with each other through an adhesive.

The high frequency-use non-reciprocal circuit element according to the present invention generally includes a non-reciprocal circuit element having a high frequency-use magnetic body provided on intersecting portions of a plurality of center electrodes which are so arranged as to intersect with each other in a state being electrically insulated from each other as described above, with dc magnetic fields applied thereto by permanent magnets, such as a lumped parameter high frequency-use non-reciprocal circuit element usable in a circulator or an isolator, for example.

As hereinabove described, the high frequency-use non-reciprocal circuit element according to the present invention has such an integrated structure that the center electrode portions are included within the high frequency-use magnetic body. Therefore, it is possible to obtain a high frequency-use non-reciprocal circuit element which is extremely smaller in size as compared with a conventional high frequency-use non-reciprocal circuit element having center electrodes which are assembled by hand. Since it is possible to omit a manual assembling step in the present invention, imperfect assembling such as misregistration of the center electrodes is hardly caused and it is possible to effectively reduce the manufacturing cost.

Thus, it is possible to provide a high frequency-use non-reciprocal circuit element which is small in size and excellent in reliability at a low cost. According to the present invention, therefore, it is possible to contribute to miniaturization, generalization and cost reduction in a high frequency device which is employed for a mobile communication system.

The foregoing and other objects, features, aspects and advantages of the present invention will become more apparent from the following detailed description of the present invention when taken in conjunction with the accompanying drawings.

#### BRIEF DESCRIPTION OF THE DRAWINGS

FIG. 1 is a perspective view showing a high frequency-use non-reciprocal circuit element according to a first embodiment of the present invention;

FIG. 2 is a perspective view showing a step of preparing the high frequency-use non-reciprocal circuit element according to the first embodiment of the present invention, with a plurality of magnetic green sheets on which center electrodes are printed;

FIG. 3 is a perspective view showing a modification of the first embodiment;

FIG. 4 is a perspective view showing a second embodiment of the present invention, with cavities formed in portions of a high frequency-use magnetic body to be provided with central electrodes;

FIG. 5 is a plan view showing a third embodiment of the present invention, in a state provided with a first layer of a magnetic body;

FIG. 6 is a plan view showing the third embodiment of the present invention, with a center electrode printed on the magnetic body;

FIG. 7 is a plan view showing the third embodiment of the present invention, with another center electrode printed on another magnetic body;

FIG. 8 is a plan view showing the third embodiment of the present invention, with still another center electrode printed on still another magnetic body;

FIGS. 9(a) to 9(c) are perspective views for illustrating center electrodes employed in a fourth embodiment of the present invention respectively;

FIG. 10 is a sectional view for illustrating a step of stacking the center electrodes and magnetic green sheets for obtaining a compact in the fourth embodiment of the present invention;

FIG. 11 is a schematic block diagram for illustrating an apparatus for forming a magnetic film and a metal film for preparing a center electrode in a fifth embodiment of the present invention;

FIG. 12 is an exploded perspective view showing magnetic plates, on which center electrodes are printed,

employed in a sixth embodiment of the present invention; and

FIG. 13 is a perspective view for illustrating a step of assembling a conventional high frequency-use non-reciprocal circuit element.

#### DESCRIPTION OF THE PREFERRED EMBODIMENTS

Description is now made on embodiments of the inventive high frequency-use non-reciprocal circuit element with reference to the drawings, thereby clarifying the present invention.

##### First Embodiment

FIG. 1 is a perspective view showing a high frequency-use non-reciprocal circuit element 1 according to a first embodiment of the present invention. The high frequency-use non-reciprocal circuit element 1 has a structure obtained by embedding a plurality of center electrodes 3a to 3c in a discoidal high frequency-use magnetic body 2 and integrating the same. The plurality of center electrodes 3a to 3c are so arranged in the high frequency-use magnetic body 2 as to intersect with each other at intervals of about 120° as shown in FIG. 1, in a state being electrically insulated from each other through magnetic layers. Both ends of the center electrodes 3a to 3c are exposed on a side surface of the high frequency-use magnetic body 2.

The high frequency-use non-reciprocal circuit element 1 is usable in a circulator or an isolator, for example. An exemplary method of manufacturing the high frequency-use non-reciprocal circuit element 1 is now described with reference to FIG. 2.

First, magnetic powder which is mainly composed of yttrium oxide ( $Y_2O_3$ ) and iron oxide ( $Fe_2O_3$ ) is mixed with an organic binder and an organic solvent, to obtain a magnetic slurry. The as-obtained magnetic slurry is shaped into magnetic green sheets 2a to 2c of 10 to several 10  $\mu m$  in thickness by a doctor blade coater.

Conductive paste which is prepared by mixing conductive powder of palladium or platinum with an organic solvent is printed on upper surfaces of the magnetic green sheets 2a to 2c by screen printing, thereby forming the center electrodes 3a to 3c. Thereafter the magnetic green sheets 2a to 2c are so arranged and stacked that the center electrodes 3a to 3c intersect with each other at angles of about 120°, and a proper number of magnetic green sheets provided with no center electrodes are additionally stacked on upper and lower portions of such a laminate, which in turn is pressurized along the direction of its thickness to obtain a compact. Then, the as-obtained compact is fired in a furnace at a temperature of 1300° to 1600° C., thereby obtaining the non-reciprocal circuit element 1 having the magnetic body 2 and the center electrodes 3a to 3c embedded therein.

In the non-reciprocal circuit element 1 according to this embodiment, the plurality of center electrodes 3a to 3c are formed by printing conductive paste on the upper surfaces of the magnetic green sheets 2a to 2c while these center electrodes 3a to 3c are electrically insulated from each other by magnetic layers formed by the magnetic green sheets 2a to 2b, as hereinabove described. Thus, it is possible not only to omit an operation of manually assembling a plurality of center electrode portions, but to position the plurality of center electrodes 3a to 3c in high accuracy. Therefore, it is possible to manufacture the high frequency-use non-reciprocal

circuit element 1, which is smaller in size than and superior in reliability to the prior art, at a low cost.

In the high frequency-use non-reciprocal circuit element 1 according to the first embodiment, the plurality of center electrodes 3a to 3c are covered with the discoidal high frequency-use magnetic body 2 to intersect with each other in a state being electrically insulated from each other through the magnetic layers. Alternatively, the high frequency-use non-reciprocal circuit element according to the first embodiment can be 10 formed to have another shape and another circuit structure.

For example, a plurality of center electrodes 3a to 3c may be arranged in a high frequency-use magnetic body 2, which is in the form of a rectangular plate, to intersect with each other in a state being electrically insulated from each other through magnetic layers, and 15 capacitance electrodes 4a to 4c forming capacitors which are electrically connected with the center electrodes 3a to 3c may be embedded in the high frequency-use magnetic body 2 to attain an integral structure including matching capacitors, as shown in FIG. 3.

Referring to FIG. 3, numerals 5a to 5f respectively denote terminal electrodes, which are formed on both side surfaces of the high frequency-use magnetic body 2 being in the form of a rectangular plate, to be electrically connected to both ends of the plurality of center electrodes 3a to 3c.

The magnetic green sheets 2a to 2c may be molded by a method such as extrusion molding, for example, in place of using the doctor blade coater. Further, the center electrodes 3a to 3c may also be formed by a method such as gravure transfer, for example, in place of screen printing.

#### Second Embodiment

Referring to FIG. 4, a method of manufacturing a high frequency-use non-reciprocal circuit element according to a second embodiment of the present invention is now described, to clarify the structure of the 40 non-reciprocal circuit element according to this embodiment.

First, magnetic green sheets identical to the magnetic green sheets 2a to 2c shown in FIG. 2 are so prepared that not conductive paste but paste containing an inflammable material such as carbon paste, which is decomposed or burned to be vanished in firing of the magnetic green sheets, or paste of a mixture of such an inflammable material and magnetic powder is printed on upper surfaces of the magnetic green sheets in the 45 same form as the center electrodes 3a to 3c.

Then, the magnetic green sheets are so stacked that the paste members printed in the form of center electrodes intersect with each other, and proper numbers of magnetic green sheets having no printed electrodes are 50 stacked on upper and lower portions of the laminate and compression-bonded along the direction of thickness to obtain a compact. Thereafter the compact is fired in a firing furnace at a temperature of 1300° to 1600° C., thereby obtaining a cylindrical high frequency-use magnetic body 2 shown in FIG. 4.

In the high frequency-use magnetic body 2, cavities 2d, 2e and 2f are defined in portions on which the paste of the aforementioned inflammable material or the mixture of the inflammable material and magnetic powder 55 has been printed. Namely, sidewardly exposed cavities 2d to 2f are formed in portions to be provided with center electrodes.

Then, the high frequency-use magnetic body 2 is dipped in a vessel storing a metal having a low melting point such as lead, tin or an alloy thereof in a molten state and pressurized, so that the cavities 2d to 2f are 5 filled up with the molten metal. Thereafter the high Frequency-use magnetic body 2 is taken out from the vessel and naturally cooled, thereby forming center electrodes in the portions provided with the cavities 2d to 2f.

Through the aforementioned steps, it is possible to obtain a structural body which is similar in structure to the high frequency-use non-reciprocal circuit element 1 shown in FIG. 1, with a plurality of center electrodes 3a to 3c embedded in and integrated with the high frequency-use magnetic body 2. Thus, it is possible to manufacture a miniature high frequency-use non-reciprocal circuit element having high reliability, similarly to the first embodiment.

#### Third Embodiment

Referring to FIGS. 5 to 8, a method of manufacturing a high frequency-use non-reciprocal circuit element according to a third embodiment of the present invention is now described, to clarify the structure of the high frequency-use non-reciprocal circuit element according to this embodiment.

First, magnetic powder which is mainly composed of yttrium oxide (Y<sub>2</sub>O<sub>3</sub>) and iron oxide (Fe<sub>2</sub>O<sub>3</sub>) is mixed with an organic binder and an organic solvent, to obtain magnetic paste. This magnetic paste is applied onto a film of synthetic resin such as polyester, for example, and dried to form a magnetic body 6a shown in FIG. 5.

Then, conductive paste prepared by mixing palladium powder and an organic solvent is applied onto the magnetic body 6a as shown in FIG. 6, to form a center electrode 7a and dry the same. Further, magnetic paste is applied onto the magnetic body 6a and the center electrode 7a again and dried to form a magnetic body 6b shown in FIG. 7. Then, conductive paste is applied onto the magnetic body 6b again and dried to form a center electrode 7b.

Further, magnetic paste is applied onto the magnetic body 6b and the center electrode 7b again as shown in FIG. 8 and dried to form a magnetic body 6c, and conductive paste is applied onto the same and dried to form a center electrode 7c. Thereafter magnetic paste is applied onto the magnetic body 6c and the center electrode 7c and dried to obtain a compact so that intersecting portions of the center electrodes 7a to 7c are located on its center.

The as-obtained compact is fired at a temperature of 1300° to 1600° C., thereby obtaining a high frequency-use non-reciprocal circuit element having a similar structure to the high frequency-use non-reciprocal circuit element 1 shown in FIG. 1.

In the third embodiment, as hereinabove described, magnetic films and center electrodes are alternately applied or printed, dried and stacked to obtain a laminate, which in turn is fired similarly to the first embodiment to obtain a high frequency-use non-reciprocal circuit element comprising a plurality of center electrodes embedded in and integrated with a high frequency-use magnetic body.

Also according to the third embodiment, therefore, it is possible to manufacture a high frequency-use non-reciprocal circuit element which is smaller in size and higher in reliability than the prior art at a low cost.

While the magnetic layer 6a is formed by applying magnetic paste and drying the same in the third embodiment, the magnetic layer 6a may be replaced by a magnetic green sheet which is employed in the first or second embodiment, so that the center electrodes and the remaining magnetic layers are formed thereon by application or printing, to obtain a laminate.

#### Fourth Embodiment

As shown in FIGS. 9(a) to 9(c), prepared are three center electrodes 8 to 10 having top plate portions 8a to 10a and pairs of side plate portions 8b, 9b and 10b downwardly extending from both ends of the top plate portions 8a to 10a. As clearly understood from FIGS. 9(a) to 9(c), the lengths of the side plate portions 8b, 9b and 10b are successively increased from the center electrode 8 toward the center electrode 10.

Then, a molding die 11 having an upwardly opening drag 11a and a cope 11b is so prepared that magnetic green sheets 2a to 2c, which are similar to those in the first embodiment but having no center electrodes printed on upper surfaces thereof, are inserted in the drag 11a alternately with the center electrodes 8 to 10 and a proper number of magnetic green sheets are inserted on the uppermost part, and the cope 11b is downwardly moved to compress the laminate, thereby obtaining a compact.

Then, the as-obtained compact is fired at a temperature of 1300° to 1600° C., to obtain a high frequency-use non-reciprocal circuit element, which is similar in structure to the high frequency-use non-reciprocal circuit element 1 shown in FIG. 1.

While the center electrodes 8 to 10 are previously formed by working metal plates in the fourth embodiment of the present invention as hereinabove described, it is possible to obtain the high frequency-use non-reciprocal circuit element 1 having the center electrodes 8 to 10 which are embedded in and integrated with a high frequency-use magnetic body by stacking the center electrodes 8 to 10 alternately with the magnetic green sheets as described above.

Also in the high frequency-use non-reciprocal circuit element according to the fourth embodiment, therefore, a high frequency-use magnetic body is homogeneously arranged around the center electrodes 8 to 10 in high density and the compact is obtained through the molding die 11, whereby it is possible to obtain a miniature high frequency-use non-reciprocal circuit element having excellent reliability. Further, the compact of the center electrodes 8 to 10 and the magnetic green sheets is manufactured through the molding die 11, whereby it is possible to manufacture the high frequency-use non-reciprocal circuit element at a lower cost as compared with a conventional method of manually assembling center electrodes, a high frequency-use magnetic body and an insulating film.

Also in the fourth embodiment, the magnetic green sheets may be replaced by the magnetic paste employed in the second embodiment. In other words, the magnetic paste may be injected after the center electrodes 8 to 10 are inserted in the die 11. In addition, the magnetic green sheets may be replaced by magnetic powder.

#### Fifth Embodiment

Referring to FIG. 11, a method of manufacturing a high frequency-use non-reciprocal circuit element according to a fifth embodiment of the present invention is now described, to clarify the high frequency-use non-

reciprocal circuit element according to this embodiment.

Referring to FIG. 11, a vacuum deposition substrate 13 of a copper plate, for example, is arranged in a vacuum vessel 12 of a sputtering unit to face a sintered body target 14 of yttrium iron garnet, for example, at a prescribed distance. Then, a magnetic film of the same composition as the target 14 is formed on a surface of the vacuum deposition substrate 13 by sputtering. Then, the as-formed magnetic film is coated with a mask 15 covering portions other than that to be provided with a center electrode, and another target of a conductive material such as copper is arranged in place of the sintered body target 14 and subjected to sputtering, to be provided with a center electrode. The steps of forming a magnetic film and a center electrode by sputtering are so repeated that it is possible to obtain an integral structural body having center electrodes embedded in a magnetic body, as shown in FIG. 11.

According to this embodiment, magnetic films and center electrodes are stacked/formed by sputtering as hereinabove described, whereby it is possible to manufacture a miniature high frequency-use non-reciprocal circuit element having high reliability at a low cost, similarly to the first embodiment.

The vacuum deposition substrate 13 can be directly applied to an earth electrode for forming an actual non-reciprocal circuit element.

While the magnetic films and the center electrodes are formed by sputtering in the fifth embodiment, it is also possible to employ another thin film forming technique such as ion plating, thermal spraying, an ion beam method, vapor deposition or vacuum deposition, to form a high frequency-use non-reciprocal circuit element in a similar manner to the above. When magnetic films are formed by such a thin film forming method, oxide magnetic films may be formed by oxidizing a metal.

#### Sixth Embodiment

FIG. 12 is an exploded perspective view for illustrating a high frequency-use non-reciprocal circuit element according to a sixth embodiment of the present invention. According to this embodiment, three magnetic plates 16a, 16b and 16c are prepared as shown in the figure. Each of the magnetic plates 16a to 16c is obtained by stacking a plurality of magnetic green sheets prepared in the first embodiment, working the same into proper dimensions and thereafter firing the same at a temperature of 1300° to 1600° C.

After the magnetic plates 16a to 16c are obtained by such firing, conductive paste which is prepared by mixing silver powder and an organic solvent, for example, is printed on the magnetic plates 16a to 16c, to form center electrodes 17a to 17c. The center electrodes 17a to 17c are so printed as to pass through centers of the discoidal magnetic plates 16a to 16c and radially extend along the same.

Then, the magnetic plates 16a to 16c are so arranged as to direct the center electrodes 17a to 17c as shown in FIG. 12 respectively, and paste containing lead borosilicate glass or the like serving as a bonding agent is applied between the magnetic plates 16a to 16c, which in turn are stacked and fired at a temperature of 900° to 1000° C. Through such firing, it is possible to obtain a high frequency-use non-reciprocal circuit element, in which a plurality of center electrodes are embedded and

integrated with each other similarly to the high frequency-use non-reciprocal circuit element shown in FIG. 1.

Also according to this embodiment, a plurality of center electrodes and high frequency-use magnetic bodies are formed by stacking fired magnetic plates 16a to 16c and integrally firing the same. Thus, it is possible to manufacture a miniature high frequency-use non-reciprocal circuit element having high reliability, similarly to the first embodiment.

Although each of the magnetic plates 16a to 16c is prepared by stacking a plurality of magnetic green sheets and firing the same in this embodiment, such magnetic plates 16a to 16c may alternatively be formed by press-molding magnetic powder.

Although the present invention has been described and illustrated in detail, it is clearly understood that the same is by way of illustration and example only and is not to be taken by way of limitation, the spirit and scope of the present invention being limited only by the terms of the appended claims.

What is claimed is:

1. A high-frequency-use non-reciprocal circuit element comprising:
  - a high-frequency-use magnetic body comprising high-frequency-use magnetic layers; and
  - a plurality of center electrodes, at least one of said center electrodes being embedded within said high-frequency-use magnetic body to make an integrated structure therewith, said center electrodes being so arranged as to intersect with each other at a junction, and being electrically insulated from each other;
2. A high frequency-use non-reciprocal circuit element in accordance with claim 1, further comprising capacitive electrodes, which are arranged in said high frequency-use magnetic body to be separated from said center electrodes by magnetic layers for forming matching electrostatic capacitance.
3. A high-frequency-use non-reciprocal circuit element in accordance with claim 1, wherein said center electrodes define equal angles with respect to each other when said plurality of center electrodes are viewed through a thickness direction of said high-frequency-use magnetic body.
4. A high-frequency-use non-reciprocal circuit element in accordance with claim 1, wherein at least two of said plurality of center electrodes are embedded within said high-frequency-use magnetic body.
5. A high-frequency-use non-reciprocal circuit element in accordance with claim 4, wherein all of said plurality of center electrodes are embedded within said high-frequency-use magnetic body.
6. A high-frequency-use non-reciprocal circuit element comprising:
  - a high-frequency-use magnetic body; and
  - a plurality of center electrodes being included in said high-frequency-use magnetic body to make an integrated structure therewith, said center electrodes being so arranged as to intersect with each other in a state being electrically insulated from each other, wherein said high-frequency-use magnetic body comprises a cofired plurality of stacked and laminated magnetic green sheets having paste members containing a material capable of being removed by sintering, being printed in correspondence to shapes of said center electrodes, said center electrodes comprising metal injected in cavities defined in the body corresponding to locations of said paste members.

7. A high-frequency-use non-reciprocal circuit element in accordance with claim 6, wherein said conductive paste is printed on said cofired plurality of stacked and laminated magnetic green sheets by forming paste members which contain a material capable of being removed by sintering, and which are printed in correspondence to shapes of said center electrodes, and wherein said center electrodes comprise metal injected in cavities defined in the body corresponding to locations of said paste members.

8. A high-frequency-use non-reciprocal circuit element in accordance with claim 6, further comprising capacitive electrodes, which are arranged in said high frequency-use magnetic body to be separated from said center electrodes by magnetic layers for forming matching electrostatic capacitance.

9. A high-frequency-use non-reciprocal circuit element in accordance with claim 6, wherein said center electrodes define equal angles with respect to each other when said plurality of center electrodes are viewed through a thickness direction of said high-frequency-use magnetic body.

10. A high-frequency-use non-reciprocal circuit element in accordance with claim 6, wherein said high frequency-use magnetic body is formed by connecting a plurality of sintered magnetic plates with each other.

11. A high-frequency-use non-reciprocal circuit element in accordance with claim 10, wherein said center electrodes are formed on single major surfaces of said magnetic plates.

12. A high-frequency-use non-reciprocal circuit element in accordance with claim 6, wherein at least two of said plurality of center electrodes are embedded within said high-frequency-use magnetic body.

13. A high-frequency-use non-reciprocal circuit element in accordance with claim 12, wherein all of said plurality of center electrodes are embedded within said high-frequency-use magnetic body.

14. A high-frequency-use reciprocal circuit element comprising:

a high-frequency-use magnetic body; and  
 a plurality of center electrodes being included in said high-frequency-use magnetic body to make an integrated structure therewith, said center electrodes being so arranged as to intersect with each other in a state being electrically insulated from each other, wherein said high-frequency-use magnetic body comprises a cofired plurality of stacked and laminated magnetic green sheets having paste members containing a material capable of being removed by sintering, being printed in correspondence to shapes of said center electrodes, said center electrodes comprising metal injected in cavities defined in the body corresponding to locations of said paste members.

15. A high-frequency-use non-reciprocal circuit element in accordance with claim 14, further comprising capacitive electrodes, which are arranged in said high frequency-use magnetic body to be separated from said center electrodes by magnetic layers for forming matching electrostatic capacitance.

16. A high-frequency-use non-reciprocal circuit element in accordance with claim 14, wherein said center electrodes define equal angles with respect to each other when said plurality of center electrodes are viewed through a thickness direction of said high-frequency-use magnetic body.

17. A high frequency-use non-reciprocal circuit element in accordance with claim 14, wherein said high frequency-use magnetic body is formed by connecting a plurality of sintered magnetic plates with each other.

18. A high frequency-use non-reciprocal circuit element in accordance with claim 17, wherein said center electrodes are formed on single major surfaces of said magnetic plates.

19. A high-frequency-use non-reciprocal circuit element in accordance with claim 14, wherein at least two of said plurality of center electrodes are embedded within said high-frequency-use magnetic body.

5 20. A high-frequency-use non-reciprocal circuit element in accordance with claim 19, wherein all of said plurality of center electrodes are embedded within said high-frequency-use magnetic body.

\* \* \* \* \*

10

15

20

25

30

35

40

45

50

55

60

65